

Dec. 4, 1928.

1,693,825

E. R. STOEKLE

RESISTANCE UNIT

Filed March 26, 1925

Fig. 1.



Fig. 2.



Fig. 3.



Fig. 4.



INVENTOR.  
Erwin R. Stoeckle  
BY ~~Franklin Hubbard~~  
ATTORNEY.

## UNITED STATES PATENT OFFICE.

ERWIN R. STOEKLE, OF MILWAUKEE, WISCONSIN, ASSIGNOR TO THE CUTLER-HAMMER MFG. CO., OF MILWAUKEE, WISCONSIN, A CORPORATION OF WISCONSIN.

## RESISTANCE UNIT.

Application filed March 26, 1925. Serial No. 18,389.

This invention relates to resistance units, and more particularly to units having a relatively large negative temperature coefficient of resistance.

5 In certain devices, such as automatic motor starters and in relays for farm lighting systems, it is desirable to include relatively high resistance in circuit initially and to automatically and rapidly decrease such resistance.

An object of this invention is to provide a resistance unit having characteristics such as to insure the aforementioned desirable results.

15 Another object is to provide an improved material having a large negative temperature coefficient of resistance.

Another object is to provide novel means for utilizing the aforementioned characteristics of said material.

Another object is to provide a resistance unit of the aforementioned character which is rugged and durable in construction.

Other objects and advantages of the invention will hereinafter appear.

I have found that iron, copper and other metals when mixed or incorporated with low melting point glasses or enamels and melted in a flame or furnace will produce a resultant mass of any desired resistance, depending upon the proportions of the respective ingredients; whereas by suitable proportioning a material may be obtained having a negative temperature coefficient of resistance such that the resistance thereof will change 300 to 400 per cent with a temperature change of 75 degrees C.

An enamel suitable for present purposes may comprise the following ingredients:

|            | Parts<br>by weight. |
|------------|---------------------|
| Red lead   | 228                 |
| Zinc oxide | 80                  |
| Raw kaolin | 35                  |
| Boric acid | 126                 |

45 These ingredients are fused together in a crucible, forming a lumpy mass, which may be partially disintegrated by immersing the same in water. The water is then removed and the material may be reduced to the desired form by grinding it in a ball mill. To a given quantity of this material I may add an equal amount by weight of iron filings or iron oxide to produce a mixture which is soft and plastic at 500 to 600 degrees C. and flows

at 1000 degrees C. If the metal is introduced in the form of an oxide, a small amount of carbon should be mixed therewith so that under the heat treatment imposed the oxide will be reduced to metallic form.

60 While I have mentioned an enamel having a particular composition it will be understood that other suitable types of enamel, or even certain forms of low melting point glass may be employed; whereas copper or other 65 suitable metals or their oxides may be substituted for that recited in the foregoing example.

I have devised a resistance unit utilizing the aforescribed material which has the 70 characteristic of reducing its resistance due to the heating effect of the current passing through it,—that is to say, a negative temperature-resistance characteristic. One form of this unit is illustrated in Fig. 1 of the accompanying drawing:

Fig. 2 illustrates a modified form of resistance unit, and

Figs. 3 and 4 show the current-resistance and temperature-resistance curves of given 80 units constructed in accordance with Figs. 1 and 2, respectively.

As illustrated in Fig. 1 a single coil 10 of resistance wire is wound upon a tubular base 11 of porcelain or other suitable material. 85 The opposite ends 12 and 13 of coil 10 are attached to conductors 14 and 15 in any suitable manner, as by soldering or brazing the former at points 16 and 17 to loops 18 and 19 of the latter, the base 11 being provided with 90 annular grooves 20 and 21 to receive said loops. The coil 10 is then coated with a layer 22 of the aforescribed high temperature coefficient of resistance material. This coating may be applied by moistening the 95 pulverized mixture with water and plastering it over the winding. The unit is then heated to about 1000 degrees C. in a furnace, so that the constituents of the coating material are fused together to form a solid mass. 100 If desired, the surface of the coating may be smoothed with a piece of graphite while the material is still in a plastic state. Upon cooling, the coating material is in the form of a stony mass having a dull grey metallic lustre. It does not crack or check, even when 105 repeatedly heated and cooled.

In Fig. 3 the curve 23 illustrates the current-resistance characteristics of a device constructed in accordance with Fig. 1 hav- 110

ing a winding of 500 ohms resistance before coating, and having a coating comprising equal parts by weight of iron filings and enamel, as heretofore described. The curve 24 5 in Fig. 3 illustrates the temperature-resistance characteristics of the same unit.

In the modified form of unit illustrated in Fig. 2, the tubular insulating base 11 is provided with two separate windings 25 and 10 26, the coils of which are parallel to but spaced from each other on said base. One end of the winding 25 leads off, as indicated at 27, whereas the other end thereof is provided with a loop 28 engaging the groove 21 15 in base 11. Similarly, the winding 26 leads off, as indicated at 29, whereas the other end thereof is looped at 30 within groove 20. The coils 25 and 26 are coated with a layer 22 of the resistance material in the manner described in connection with Fig. 1.

The current-resistance and temperature-resistance curves of a device constructed in accordance with Fig. 2 are illustrated at 31 and 32, respectively, in Fig. 4. As indicated by said curves, the device of Fig. 2 provides a comparatively low initial resistance which, moreover, decreases rapidly. This low resistance is due to the fact that the current paths are between the adjacent wires of the 30 winding along their full length.

As will be obvious, the resistance characteristics of the devices may be varied by changing the proportion of conducting substance in the composite resistance material, whereas the 35 initial resistance of a device like that shown in Fig. 1 can be predetermined by using a wire of a given resistance value. Various other modifications will be obvious from the above description or will be apparent to those 40 skilled in the art. I therefore do not desire to be limited to the particular embodiments of my invention shown herein, which merely indicate the broad range of applicability of the invention.

45 What I claim and desire to secure by Letters Patent is:

1. A resistance unit comprising a resistance winding and a body of normally slightly

conductive resistance material adapted to embed the same, said material comprising a mixture of finely divided iron and a finely divided vitreous substance in jointly fused condition. 50

2. A resistance unit comprising a winding of predetermined resistance, the coils of said winding being embedded in a resistance material consisting of substantially equal parts of a metallic substance and an enamel composed of red lead, zinc oxide, raw kaolin and boric acid. 55

3. A resistance unit comprising a winding of predetermined resistance, said winding being embedded in a fused compound consisting of equal parts of iron filings and an enamel, said enamel having ingredients in the following proportions by weight: 60

|            |     |
|------------|-----|
| Red lead   | 228 |
| Zinc oxide | 80  |
| Raw kaolin | 35  |
| Boric acid | 126 |

70

4. A resistance unit comprising a tubular insulating core, a resistance wire wound thereabout, and a body of normally slightly conductive resistance material surrounding said wire and embedding the same, said resistance material having a negative temperature coefficient of resistance and comprising a mixture of substantially equal parts of iron filings and a finely divided vitreous enamel in jointly fused condition. 75

5. A resistance unit comprising an insulating core, a plurality of resistance wires wound thereabout, the coils of said wires being arranged in parallel spaced relation to each other throughout the length thereof, and a body of normally slightly conductive resistance material surrounding said coils and embedding the same, said resistance material having a negative temperature coefficient of resistance and comprising a mixture, in predetermined proportions, of iron filings and a finely divided vitreous enamel in jointly fused condition. 80

In witness whereof, I have hereunto subscribed my name.

ERWIN R. STOEKLE.